

UNITED STATES PATENT OFFICE

2.145.297

# **TREATMENT OF TEXTILE FABRICS AND THE PRODUCTS THEREOF**

**Camille Dreyfus, New York, N. Y.**

No Drawing. Application April 3, 1937,  
Serial No. 134,901

4 Claims. (Cl. 8—129)

This invention relates to the treatment of fabrics containing fibers of an organic derivative of cellulose and relates more particularly to the treatment of such fabrics with a modifying agent 5 in order to impart to the fabrics a fuller, more lofty and resilient hand.

An object of the invention is the economical and expeditious method of treating a fabric, containing at least some yarns formed of a mixture of fibers of organic derivatives of cellulose and animal fibers, to impart to the fabric a resilient, full and voluminous hand. Another object of the invention is the treatment of fabrics, containing both animal fibers and fibers of an organic derivative of cellulose, to impart a desired hand thereto without reducing the strength or other properties of the animal fibers. Other objects of the invention will appear from the following detailed description.

described.

20 It is known that fabrics containing a mixture of animal fibers and artificial fibers or filaments containing organic derivatives are made by a variety of processes. These fabrics, however, although they may have the desired appearance and 25 strength often do not have the desired hand or feel. In some instances fabrics, made of yarns containing animal fibers and fibers of an organic derivative of cellulose, which are intended to compete commercially with fabrics of all-animal 30 fibers, have a rag-like or boardy hand, whereas the fabric of all-animal fibers of the same structure has a resilient feel and is lofty in hand. By treating, in accordance with this invention, a fabric which has a rag-like hand comprising 35 fibers or filaments of organic derivatives of cellulose and animal fibers, the treated fabric is in all respects similar to the fabric of the same construction formed entirely of animal fibers.

A further advantage of treating fabrics in accordance with this invention is that the fabrics so treated have the property of a non-slipping fabric, that is, the warp and weft appear to be anchored to each other, and even in fairly open fabric or loosely woven fabric the tendency of the weft to slip on the warp is greatly reduced.

45 went to strip off the warp is greatly reduced.  
The modifying agents usually applied to fabrics, made of or containing both organic derivative of cellulose and animal fibers, to modify the hand of the same often have a detrimental effect  
50 on one or the other of the fibers. Some modifying agents destroy or at least deaden the resiliency or "life" of the animal fibers, while others make the animal fibers brittle and still others change the dye affinity of the organic derivative of cellulose or reduce its strength, elongation properties,  
55

etc. The treatment of fabrics in accordance with this invention obviates these detrimental effects.

The treatment of fabrics, made from or containing yarns composed of animal fibers and fibers or filaments of an organic derivative of cellulose, tends to produce a heavier animal fiber cover on the surface than the fabric had prior to treatment. This lends to the fabric a touch more nearly that of a fabric made wholly of animal fibers. 10

In accordance with my invention, I treat fabrics made of animal fibers and organic derivative of cellulose fibers or filaments with a modifying agent comprising an ammonium alkali metal or alkaline earth metal salt of thiocyanic acid in an aqueous solution or emulsion. The time of treatment, temperature of treatment and the concentration of the thiocyanate set forth below are critical as more strenuous treatments tend to weaken the fabric, while less strenuous treatments, although they do not injure the fabric, do not produce sufficient improvement in the hand of the fabric to be classed commercially beneficial. The modifying agent may contain, besides the thiocyanate and water, oily materials such as sulphonated or sulphated fatty alcohols, vegetable or mineral oils, wool fat or oil, etc., that give a "live" resilient feeling to the fabric.

The fabric to be treated by my invention may be any suitable woven, knitted, netted or knotted fabric. This fabric contains at least some yarns formed from a mixture of fibers of organic derivatives of cellulose and other fibers. Any suitable organic derivative of cellulose, such as the organic esters of cellulose and the cellulose ethers, may be employed for forming a part of the fibers. Examples of the organic esters of cellulose are cellulose acetate, cellulose formate, cellulose propionate and cellulose butyrate, while examples of the cellulose ethers are ethyl cellulose, methyl cellulose and benzyl cellulose.

While the best results are obtained by the treatment of fabrics which consist wholly of yarns containing fibers of organic derivatives of cellulose and animal fibers, novel effects may be obtained by the treatment of fabrics that contain, besides such yarns, other types of yarns such as those formed from continuous filaments of organic derivatives of cellulose or yarns formed from silk, reconstituted or regenerated cellulose, animal fibers or mixtures of these. Fabrics may also be formed by interweaving or knitting yarns containing organic derivatives of cellulose fibers with yarns formed entirely of animal fibers with or without other types of yarns being present. 55

- The artificial fibers containing organic derivatives of cellulose employed in forming at least some of the yarns in the fabric may be made by any suitable method, for example, by extruding 5 an organic ester of cellulose dissolved in a volatile solvent through suitable orifices into a solidifying medium, thus forming substantially continuous filaments. A plurality of these filaments as they are formed, or from a plurality of preformed 10 packages, may be grouped together in the form of a rope or they may be formed into a band, then cut or torn to staple lengths. Either the continuous filaments before reduction to staple fiber or the staple fibers may be treated by applying thereto effect materials, lubricants, or other finishes and they may or may not be embossed to form crimps therein or treated in baths which cause the fibers to curl. Fibers from 1 to 12 or 15 more inches in length may be employed to form the yarns. These artificial fibers may be mixed with wool, alpaca, camel hair or other animal fibers and processed into threads or yarns by the woolen method, the cotton method, the waste silk method or other suitable methods.
- 20 The yarns may be formed of a mixture of from 50 to 5 parts of organic derivative of cellulose fibers and from 5 to 50 parts of animal fibers. The yarns may also contain other fibers and filaments such as cotton, regenerated cellulose, etc.
- 25 For forming fabrics suitable for men's wear which have the appearance and hand of all-wool worsted fabrics, it is preferable to form the yarn from about 70 parts of cellulose acetate fibers and about 30 parts of wool fibers. For other types of 30 fabrics other percentages may be more desirable.

The modifying agent with which the fabrics are to be treated preferably is an aqueous solution of an ammonia, an alkali metal or an alkaline earth metal salt of thiocyanic acid of from 6° to 40 10° Bé. The term "alkali salt of thiocyanic acid" used in the claims includes any such salts. Mixtures of such salts may also be employed. When treating fabrics so constructed that they rely upon the properties of animal fibers for hand or appearance, the concentration of the thiocyanic acid salt in the modifying agent is preferably below 10° Bé. and the period and temperature of treatment are such that there is no tendency for the modifying agent to extract the oil from the animal fibers or otherwise modify the animal 45 fibers to render the same more brittle.

50 Any suitable fabric as described above may be treated with the modifying agent by submerging the fabric in a bath of the modifying agent, which bath is maintained at a temperature between 10 and 13° C., depending upon the duration of the treatment and upon the concentration of the salt of thiocyanic acid in the bath. When treating fabrics containing 70 parts cellulose acetate and about 30 parts of wool dispersed in each other and formed into yarns a temperature of from 11° to 12° C. is preferred.

55 The time of treatment will depend upon the concentration of the salt of thiocyanic acid and upon the temperature at which the treatment is carried out. With the concentrations and temperatures set forth above, the duration of treatment is preferably from 4 to 6 minutes.

60 After treatment of the fabric with the modifying agent the excess modifying agent may be removed from the fabric by passing the same through nip rollers or through a pair of rollers covered with an absorbent material such as linen or cotton fabric, the rolls being at room temperature or at elevated temperatures. Or the fabric,

65 after removal from the bath containing the modifying agent, may be immediately immersed in one or more rinsing baths to remove the modifying agents.

70 As a guide to the concentrations of modifying agents, temperatures and time of treatment which may be employed in accordance with this invention, the following table is given—the fabric being treated consisting of about 70 parts cellulose acetate fibers and about 30 parts animal 10 fibers, while the modifying agent is ammonium thiocyanate:

75  $6\frac{1}{2}$ – $7\frac{1}{2}$ ° Bé. at 13–11° C. for 4 to 6 minutes  
 $9\frac{1}{2}$ ° Bé. at 11–10° C. for 4 to 6 minutes

80 To further illustrate the invention, the following examples are given:

85 *Example I*

90 A fabric consisting of yarns made of about 70 parts cellulose acetate fibers and about 30 parts animal fibers are treated for 5 minutes at 12° C. in a bath containing ammonium thiocyanate of 7° Bé. The fabric, after removal from the modifying bath, is immediately rinsed to remove substantially all the modifying agent therefrom. The fabric treated had 45 ends and 40 picks when dyed, scoured and finished in the regular manner, while after dyeing, scouring and finishing and also with the treatment of this example the fabric had 47 ends and 43 picks. The fabric so treated has a resilient, full and voluminous hand.

95 *Example II*

100 A fabric consisting of 70 parts cellulose acetate fibers and about 30 parts of wool fibers is treated for 5 minutes at 11° C. in an aqueous solution of ammonia thiocyanate of  $9\frac{1}{4}$ ° Bé. The fabric when regularly dyed, scoured and finished has 45 ends and 40 picks, while after treatment in accordance with this example, then dyed, scoured and finished has 50 ends and 48 picks. The fabric so treated has a resilient, full and voluminous hand.

105 The treatment in accordance with this invention may be performed upon the fabric prior to dyeing or after dyeing and prior to finishing, it being preferable, however, to treat the fabric in accordance with this invention prior to dyeing as the thiocyanate salts in some cases have a tendency to modify colors and dyes.

110 It is to be understood that the foregoing detailed description is given merely by way of illustration and that many variations may be made therein without departing from the spirit of my invention.

115 Having described my invention, what I desire to secure by Letters Patent is:

120 1. Process for the production of improved textile fabrics, which comprises treating a fabric, containing yarns formed from fibers some of which are composed of an organic derivative of cellulose and some of which are animal fibers, at 10 to 13° C. for 6 minutes or less with an aqueous solution of an alkali salt of thiocyanic acid having a density of 6 to 10° Bé.

125 2. Process for the production of improved textile fabrics, which comprises treating a fabric, containing yarns formed from fibers some of which are composed of cellulose acetate and some of which are animal fibers, at 10 to 13° C. for 6 minutes or less with an aqueous solution of an alkali salt of thiocyanic acid having a density of 6 to 10° Bé.

5 3. Process for the production of improved textile fabrics, which comprises treating a fabric, containing yarns formed from fibers some of which are composed of an organic derivative of cellulose and some of which are animal fibers, at 10 to 13° C. for 4 to 6 minutes with an aqueous solution of ammonium thiocyanate having a density of 6 to 10° Bé.

4. Process for the production of improved textile fabrics, which comprises treating a fabric, containing yarns formed from fibers some of which are composed of cellulose acetate and some of which are animal fibers, at 10 to 13° C. for 4 to 5 minutes with an aqueous solution of ammonium thiocyanate having a density of 6 to 10° Bé.

CAMILLE DREYFUS.